



US010907234B2

(12) **United States Patent**  
**Fujimura et al.**

(10) **Patent No.:** **US 10,907,234 B2**  
(45) **Date of Patent:** **Feb. 2, 2021**

(54) **GRAIN-ORIENTED ELECTRICAL STEEL SHEET AND DECARBURIZED STEEL SHEET USED FOR MANUFACTURING THE SAME**

(71) Applicant: **NIPPON STEEL & SUMITOMO METAL CORPORATION**, Tokyo (JP)

(72) Inventors: **Hiroshi Fujimura**, Tokyo (JP); **Fumiaki Takahashi**, Tokyo (JP); **Takashi Kataoka**, Tokyo (JP)

(73) Assignee: **NIPPON STEEL CORPORATION**, Tokyo (JP)

(\*) Notice: Subject to any disclaimer, the term of this patent is extended or adjusted under 35 U.S.C. 154(b) by 306 days.

(21) Appl. No.: **15/768,696**

(22) PCT Filed: **Oct. 26, 2016**

(86) PCT No.: **PCT/JP2016/081732**

§ 371 (c)(1),

(2) Date: **Apr. 16, 2018**

(87) PCT Pub. No.: **WO2017/073615**

PCT Pub. Date: **May 4, 2017**

(65) **Prior Publication Data**

US 2018/0305784 A1 Oct. 25, 2018

(30) **Foreign Application Priority Data**

Oct. 26, 2015 (JP) ..... 2015-209663

(51) **Int. Cl.**

**C21D 9/46** (2006.01)

**C22C 38/16** (2006.01)

**H01F 1/18** (2006.01)

**C21D 8/12** (2006.01)

**C22C 38/60** (2006.01)

(Continued)

(52) **U.S. Cl.**

CPC ..... **C21D 9/46** (2013.01); **C21D 3/04** (2013.01); **C21D 6/008** (2013.01); **C21D 8/005** (2013.01);

(Continued)

(58) **Field of Classification Search**

CPC ..... C22C 38/00; C21D 8/1222  
See application file for complete search history.

(56) **References Cited**

U.S. PATENT DOCUMENTS

2009/0047537 A1 2/2009 Nanba et al.  
2015/0170812 A1\* 6/2015 Murakami ..... C22C 38/00  
148/111  
2020/0063234 A1\* 2/2020 Suehiro ..... C21D 8/1222

FOREIGN PATENT DOCUMENTS

EP 0 957 180 A2 11/1999  
EP 2 775 007 A1 9/2014  
(Continued)

OTHER PUBLICATIONS

Extended European Search Report for European Application No. 16859844.9, dated Jun. 7, 2019.

(Continued)

*Primary Examiner* — Scott R Kastler

(74) *Attorney, Agent, or Firm* — Birch, Stewart, Kolasch & Birch, LLP

(57) **ABSTRACT**

A grain-oriented electrical steel sheet includes: a chemical composition represented by, in mass %, Si: 1.8% to 7.0%, Cu: 0.03% to 0.60%, and the balance: Fe and impurities; and a primary coating film containing forsterite on a surface of the steel sheet, in which a Cu/Fe light-emitting intensity ratio at an interface region between the primary coating film and the surface of the steel sheet is 0.30 or less.

**5 Claims, 3 Drawing Sheets**



|      |                   |                                                                                                                                                                                                                                                                                                                                                                                                                                                                                     |    |               |              |        |  |
|------|-------------------|-------------------------------------------------------------------------------------------------------------------------------------------------------------------------------------------------------------------------------------------------------------------------------------------------------------------------------------------------------------------------------------------------------------------------------------------------------------------------------------|----|---------------|--------------|--------|--|
| (51) | <b>Int. Cl.</b>   |                                                                                                                                                                                                                                                                                                                                                                                                                                                                                     |    |               |              |        |  |
|      | <i>H01F 1/16</i>  | (2006.01)                                                                                                                                                                                                                                                                                                                                                                                                                                                                           | JP | 8-269552 A    | 10/1996      |        |  |
|      | <i>C21D 3/04</i>  | (2006.01)                                                                                                                                                                                                                                                                                                                                                                                                                                                                           | JP | 8-277421 A    | 10/1996      |        |  |
|      | <i>C21D 6/00</i>  | (2006.01)                                                                                                                                                                                                                                                                                                                                                                                                                                                                           | JP | 9-268322 A    | 10/1997      |        |  |
|      | <i>C21D 8/00</i>  | (2006.01)                                                                                                                                                                                                                                                                                                                                                                                                                                                                           | JP | 10-8133 A     | 1/1998       |        |  |
|      | <i>C22C 38/00</i> | (2006.01)                                                                                                                                                                                                                                                                                                                                                                                                                                                                           | JP | 10-102149 A   | 4/1998       |        |  |
|      | <i>C22C 38/02</i> | (2006.01)                                                                                                                                                                                                                                                                                                                                                                                                                                                                           | JP | 2003-193141 A | 7/2003       |        |  |
|      | <i>C22C 38/04</i> | (2006.01)                                                                                                                                                                                                                                                                                                                                                                                                                                                                           | JP | 2005-290446 A | 10/2005      |        |  |
|      | <i>C23G 1/08</i>  | (2006.01)                                                                                                                                                                                                                                                                                                                                                                                                                                                                           | JP | 2008-127634 A | 6/2008       |        |  |
| (52) | <b>U.S. Cl.</b>   |                                                                                                                                                                                                                                                                                                                                                                                                                                                                                     |    |               |              |        |  |
|      | CPC .....         | <i>C21D 8/12</i> (2013.01); <i>C21D 8/1222</i> (2013.01); <i>C21D 8/1233</i> (2013.01); <i>C21D 8/1255</i> (2013.01); <i>C21D 8/1261</i> (2013.01); <i>C21D 8/1283</i> (2013.01); <i>C22C 38/001</i> (2013.01); <i>C22C 38/002</i> (2013.01); <i>C22C 38/008</i> (2013.01); <i>C22C 38/02</i> (2013.01); <i>C22C 38/04</i> (2013.01); <i>C22C 38/16</i> (2013.01); <i>C22C 38/60</i> (2013.01); <i>C23G 1/085</i> (2013.01); <i>H01F 1/16</i> (2013.01); <i>H01F 1/18</i> (2013.01) |    | JP            | 2011-68968 A | 4/2011 |  |
|      |                   |                                                                                                                                                                                                                                                                                                                                                                                                                                                                                     | JP | 2011-111645 A | 6/2011       |        |  |
|      |                   |                                                                                                                                                                                                                                                                                                                                                                                                                                                                                     | JP | 2012-214902 A | 11/2012      |        |  |
|      |                   |                                                                                                                                                                                                                                                                                                                                                                                                                                                                                     | JP | 2014-196559 A | 10/2014      |        |  |

## OTHER PUBLICATIONS

International Preliminary Report on Patentability and English translation of the Written Opinion of the International Searching Authority (forms PCT/IB/373, PCT/ISA/237 and PCT/IB/338), dated May 11, 2018, for corresponding International Application No. PCT/JP2016/081732.

International Search Report for PCT/JP2016/081732 dated Jan. 31, 2017.

Written Opinion of the International Searching Authority for PCT/JP2016/081732 (PCT/ISA/237) dated Jan. 31, 2017.

\* cited by examiner

## References Cited

## FOREIGN PATENT DOCUMENTS

|    |           |        |
|----|-----------|--------|
| JP | 6-88171 A | 3/1994 |
| JP | 7-48674 A | 2/1995 |

FIG. 1



FIG. 2



FIG. 3



1

**GRAIN-ORIENTED ELECTRICAL STEEL  
SHEET AND DECARBURIZED STEEL  
SHEET USED FOR MANUFACTURING THE  
SAME**

**TECHNICAL FIELD**

The present invention relates to a grain-oriented electrical steel sheet and a decarburized steel sheet used for manufacturing the same.

**BACKGROUND ART**

A grain-oriented electrical steel sheet used for an iron core material of, for example, a transformer and the like is a steel sheet that contains Si of 1.8 mass % to 7 mass % or so and in which crystal grain orientations of a product are highly accumulated in the  $\{110\}<001>$  orientation. The control of these crystal orientations is achieved by utilizing a catastrophic grain growth phenomenon called secondary recrystallization. As a typical method for controlling this secondary recrystallization, there is a method in which a steel billet is heated to a high temperature of 1280° C. or more before hot rolling to once solid-dissolve precipitates such as AlN, and in a hot rolling step and a subsequent annealing step, they are made to precipitate again as fine precipitates called inhibitors. Although a lot of developments have been made in order to obtain a steel sheet having a more excellent magnetic property in the manufacture of such a grain-oriented electrical steel sheet, achievement of much lower core loss has been required as a demand for recent energy-saving further increases. Although there are various methods for achieving low core loss of the grain-oriented electrical steel sheet, a method of increasing a magnetic flux density to reduce a hysteresis loss is effective. For improving the magnetic flux density of the grain-oriented electrical steel sheet, it is important to highly accumulate crystal grain orientations of a product in the  $\{110\}<001>$  orientation. In order to highly accumulate the crystal grain orientations of a product in the  $\{110\}<001>$  orientation, various techniques regarding the grain-oriented electrical steel sheet and a chemical composition of a slab used for its manufacture have been proposed.

In the meantime, at the final stage in the manufacture of the grain-oriented electrical steel sheet, the steel sheet has an annealing separating agent containing MgO as its main component applied thereto to be dried and is coiled into a coil, and then is subjected to final finish annealing. On this occasion, due to a reaction between MgO and a coating film mainly composed of SiO<sub>2</sub> that is formed in decarburization annealing, a primary coating film containing forsterite (Mg<sub>2</sub>SiO<sub>4</sub>) as its main component is formed on the surface of the steel sheet. Thus, for utilizing such a method of improving the magnetic flux density as described above on an industrial scale, in addition to the magnetic property being good, it is important for adhesion of the primary coating film to be good stably.

Although various techniques have been proposed so far, it is difficult to achieve both a good magnetic property and excellent adhesion between the primary coating film and the steel sheet.

**CITATION LIST**

**Patent Literature**

Patent Literature 1: Japanese Laid-open Patent Publication No. 06-88171

2

Patent Literature 2: Japanese Laid-open Patent Publication No. 08-269552

Patent Literature 3: Japanese Laid-open Patent Publication No. 2005-290446

5 Patent Literature 4: Japanese Laid-open Patent Publication No. 2008-127634

Patent Literature 5: Japanese Laid-open Patent Publication No. 2012-214902

10 Patent Literature 6: Japanese Laid-open Patent Publication No. 2011-68968

Patent Literature 7: Japanese Laid-open Patent Publication No. 10-8133

15 Patent Literature 8: Japanese Laid-open Patent Publication No. 07-48674

**SUMMARY OF INVENTION**

**Technical Problem**

20 An object of the present invention is to provide a grain-oriented electrical steel sheet having a good magnetic property and having excellent adhesion between a primary coating film and the steel sheet and a decarburized steel sheet used for manufacturing the same.

25

30 The present inventors conducted earnest examinations in order to solve the above-described problems. As a result of the earnest examination, it became clear that in the case where Cu and a specific element such as Bi are contained in the steel sheet, it is possible to obtain an excellent magnetic property, but it is not possible to obtain sufficient adhesion of the primary coating film. Then, the present inventors 35 further conducted earnest examinations of the effect of Cu on the adhesion of the primary coating film. As a result, they found out that the steel sheet containing the above-described specific element and Cu and having good adhesion with the primary coating film correlates with the Cu concentration at 40 an interface region between the primary coating film and the steel sheet.

45 As a result of further repeated earnest examinations based on such findings, the present inventors have reached the following various aspects of the invention.

(1)

A grain-oriented electrical steel sheet, includes:  
a chemical composition represented by  
in mass %,  
Si: 1.8% to 7.0%,  
Cu: 0.03% to 0.60%, and  
50 the balance: Fe and impurities; and  
a primary coating film containing forsterite on a surface of  
the steel sheet, in which  
a Cu/Fe light-emitting intensity ratio at an interface region  
55 between the primary coating film and the surface of the steel sheet is 0.30 or less.

(2)

A decarburized steel sheet for a grain-oriented electrical steel sheet, includes:  
60 a chemical composition represented by  
in mass %,  
C: 0.03% to 0.15%,  
Si: 1.8% to 7.0%,  
Mn: 0.02% to 0.30%,  
65 S: 0.005% to 0.040%,  
acid-soluble Al: 0.010% to 0.065%,  
N: 0.0030% to 0.0150%,

Cu: 0.03% to 0.60%,  
 Sn: 0% to 0.5%,  
 Ge, Se, Sb, Te, Pb, or Bi, or an arbitrary combination of these: 0.0005% to 0.030% in total, and the balance: Fe and impurities; and an oxide film on a surface of the steel sheet, in which a Cu/Fe light-emitting intensity ratio at an interface region between the oxide film and the surface of the steel sheet is 0.60 or less.

(3)

A manufacturing method of a grain-oriented electrical steel sheet, includes:

a step of heating a slab in a temperature zone of 1300° C. to 1490° C.;

a step of obtaining a hot-rolled steel sheet by performing hot rolling of the slab;

a step of coiling the hot-rolled steel sheet in a temperature zone of 600° C. or less;

a step of performing hot-rolled sheet annealing of the hot-rolled steel sheet;

after the hot-rolled sheet annealing, a step of performing cold rolling and obtaining a cold-rolled steel sheet;

a step of performing decarburization annealing of the cold-rolled steel sheet; and

after the decarburization annealing, a step of applying an annealing separating agent containing MgO and performing finish annealing, in which

the step of performing the hot rolling includes a step of performing rough rolling with a finishing temperature set to 1200° C. or less and a step of performing finish rolling with a start temperature set to 1000° C. or more and a finishing temperature set to 950° C. to 1100° C.,

in the hot rolling, the finish rolling is started within 300 seconds after start of the rough rolling,

cooling at a cooling rate of 50° C./second or more is started within 10 seconds after finish of the finish rolling,

pickling with a holding temperature set to 50° C. or more and a holding time period set to 30 seconds or more is performed in a pickling bath containing a nitric acid, a pickling inhibitor, and a surface active agent after the hot rolling and before finish of the cold rolling, and

the slab includes a chemical composition represented by, in mass %,

C: 0.03% to 0.15%,

Si: 1.8% to 7.0%,

Mn: 0.02% to 0.30%,

S: 0.005% to 0.040%,

acid-soluble Al: 0.010% to 0.065%,

N: 0.0030% to 0.0150%,

Cu: 0.03% to 0.60%,

Sn: 0% to 0.5%,

Ge, Se, Sb, Te, Pb, or Bi, or an arbitrary combination of these: 0.0005% to 0.030% in total, and the balance: Fe and impurities.

(4)

The manufacturing method of the grain-oriented electrical steel sheet according to (3), in which the pickling bath further contains a nitrate.

(5)

A manufacturing method of a decarburized steel sheet for a grain-oriented electrical steel sheet, includes:

a step of heating a slab in a temperature zone of 1300° C. to 1490° C.;

a step of obtaining a hot-rolled steel sheet by performing hot rolling of the slab;

a step of coiling the hot-rolled steel sheet in a temperature zone of 600° C. or less;

a step of performing hot-rolled sheet annealing of the hot-rolled steel sheet;

after the hot-rolled sheet annealing, a step of performing cold rolling and obtaining a cold-rolled steel sheet; and

5 a step of performing decarburization annealing of the cold-rolled steel sheet; in which

the step of performing the hot rolling includes a step of performing rough rolling with a finishing temperature set to 1200° C. or less and a step of performing finish rolling with

10 a start temperature set to 1000° C. or more and a finishing temperature set to 950° C. to 1100° C.,

in the hot rolling, the finish rolling is started within 300 seconds after start of the rough rolling,

cooling at a cooling rate of 50° C./second or more is started within 10 seconds after finish of the finish rolling,

pickling with a holding temperature set to 50° C. or more and a holding time period set to 30 seconds or more is performed in a pickling bath containing a nitric acid, a pickling inhibitor, and a surface active agent after the hot rolling and before finish of the cold rolling, and

20 the slab includes a chemical composition represented by, in mass %

C: 0.03% to 0.15%,

Si: 1.8% to 7.0%,

Mn: 0.02% to 0.30%,

S: 0.005% to 0.040%,

acid-soluble Al: 0.010% to 0.065%,

N: 0.0030% to 0.0150%,

Cu: 0.03% to 0.60%,

Sn: 0% to 0.5%,

Ge, Se, Sb, Te, Pb, or Bi, or an arbitrary combination of these: 0.0005% to 0.030% in total, and the balance: Fe and impurities.

(6)

The manufacturing method of the decarburized steel sheet for a grain-oriented electrical steel sheet according to (5), in which the pickling bath further contains a nitrate.

#### Advantageous Effects of Invention

According to the present invention, it is possible to obtain excellent adhesion between a primary coating film and a steel sheet and a good magnetic property because the Cu concentration at an interface region between the primary coating film and the steel sheet is appropriate.

#### BRIEF DESCRIPTION OF DRAWINGS

50 FIG. 1 is images resulting from photographing surfaces of samples that have undergone a bending test.

FIG. 2 is a chart illustrating the relationship between a Cu concentration at an interface region between a primary coating film and a steel sheet and a minimum bend radius at which peeling occurs.

55 FIG. 3 is a chart illustrating measurement examples of an Fe light-emitting intensity, a Cu light-emitting intensity, and a Cu/Fe light-emitting intensity ratio by GDS analysis.

#### DESCRIPTION OF EMBODIMENTS

Hereinafter, there will be explained embodiments of the present invention in detail.

When manufacturing a grain-oriented electrical steel sheet using a silicon steel material that contains a specific element such as Bi for the purpose of improving a magnetic property, the adhesion between a primary coating film and the steel sheet sometimes deteriorates. Conventionally, it has

been known that Cu is contained in a slab when scrap is mixed in a raw material at the time of steelmaking, but mixture of Cu from the scrap has not been a problem in particular as long as it is small in amount because Cu is an element to improve the magnetic property and is not a particularly controversial element with respect to the adhesion of the primary coating film. However, the present

samples that have undergone the bending test of the steel sheets manufactured using Steel type MD1 to Steel type MD6. Further, measurement results of the magnetic flux density  $B_8$  are illustrated in Table 2. Incidentally, the specific element in Table 1 indicates Ge, Se, Sb, Te, Pb, or Bi, and the steel type with the description of “-” in the space of specific element used no specific element.

TABLE 1

| STEEL<br>TYPE | CHEMICAL COMPOSITION (MASS %) |     |      |       |       |        |                  |      |        |            | SPECIFIC<br>ELEMENT |
|---------------|-------------------------------|-----|------|-------|-------|--------|------------------|------|--------|------------|---------------------|
|               | C                             | Si  | Mn   | P     | S     | Cu     | ACID-<br>SOLUBLE | Al   | Sn     | N          |                     |
| MD1           | 0.08                          | 3.3 | 0.04 | 0.008 | 0.025 | <0.005 | 0.028            | 0.10 | 0.0081 | —          |                     |
| MD2           | 0.08                          | 3.3 | 0.04 | 0.008 | 0.025 | <0.005 | 0.028            | 0.10 | 0.0081 | Bi = 0.005 |                     |
| MD3           | 0.08                          | 3.3 | 0.04 | 0.008 | 0.026 | 0.410  | 0.028            | 0.10 | 0.0082 | —          |                     |
| MD4           | 0.08                          | 3.3 | 0.04 | 0.008 | 0.026 | 0.410  | 0.028            | 0.10 | 0.0083 | Te = 0.005 |                     |
| MD5           | 0.08                          | 3.3 | 0.04 | 0.008 | 0.025 | 0.800  | 0.025            | 0.10 | 0.0081 | —          |                     |
| MD6           | 0.08                          | 3.3 | 0.08 | 0.008 | 0.025 | 0.200  | 0.028            | 0.10 | 0.0080 | Pb = 0.035 |                     |
| MD7           | 0.08                          | 3.3 | 0.08 | 0.008 | 0.025 | 0.300  | 0.027            | 0.10 | 0.0080 | Ge = 0.005 |                     |
| MD8           | 0.08                          | 3.3 | 0.08 | 0.008 | 0.015 | 0.300  | 0.027            | 0.10 | 0.0080 | Se = 0.015 |                     |
| MD9           | 0.08                          | 3.3 | 0.08 | 0.008 | 0.025 | 0.300  | 0.027            | 0.10 | 0.0080 | Sb = 0.025 |                     |
| MD10          | 0.08                          | 3.3 | 0.08 | 0.008 | 0.025 | 0.400  | 0.027            | 0.10 | 0.0080 | Pb = 0.006 |                     |

inventors found out that in the case of using the silicon steel material containing the above-described specific element, the adhesion of the primary coating film deteriorates even at a level where the Cu content has been considered to be uncontroversial conventionally, a Cu concentrated portion exists on the surface of a steel sheet resulting from decarburization annealing, and this portion causes the deterioration. Then, as a result of further repeated earnest examinations, the present inventors found out that pickling under a conventional treatment condition fails to remove the Cu concentrated portion on the surface of the steel sheet, and in a manufacturing process, the Cu concentrated portion is removed from the surface of the steel sheet by pickling under a predetermined condition, thereby enabling an improvement in the adhesion of the primary coating film. Hereinafter, there will be explained an experiment by which such findings were able to be obtained.

In a vacuum melting furnace, silicon steel materials having chemical compositions illustrated in Table 1 were fabricated, after being heated at 1350° C., slabs were subjected to hot rolling to obtain hot-rolled steel sheets having a sheet thickness of 2.3 mm, and then they were subjected to hot-rolled sheet annealing and pickling and then subjected to cold rolling, and cold-rolled steel sheets having a sheet thickness of 0.22 mm were obtained. Incidentally, each balance of the silicon steel materials illustrated in Table 1 is Fe and impurities. Then, the cold-rolled steel sheets were subjected to primary recrystallization annealing including decarburization annealing, had an annealing separating agent containing MgO as its main component applied thereto, and then were subjected to finish annealing, and various grain-oriented electrical steel sheets were obtained. The obtained steel sheets had an insulating coating film applied thereto to be baked. Each magnetic flux density  $B_8$  (magnetic flux density at a magnetic field intensity of 800 A/m) of the obtained steel sheets was measured. Further, each sample was taken from a portion 50 mm away from the end in a coil width direction in the finish annealing and from a center portion in the coil width direction, and they were subjected to a bending test in which each sample was wound on a 20-mm  $\phi$  cylindrical body. The adhesion of the primary coating film was evaluated from these results. FIG. 1 shows images resulting from photographing surfaces of the

25  
30  
35

TABLE 2

| STEEL TYPE | MAGNETIC FLUX<br>DENSITY $B_8$ (T) |
|------------|------------------------------------|
| MD1        | 1.786                              |
| MD2        | 1.925                              |
| MD3        | 1.859                              |
| MD4        | 1.945                              |
| MD5        | 1.920                              |
| MD6        | 1.954                              |
| MD7        | 1.956                              |
| MD8        | 1.949                              |
| MD9        | 1.951                              |
| MD10       | 1.953                              |

40  
45  
50  
55  
60

Table 2 reveals that in Steel type MD4 and Steel type MD6 to Steel type MD10 each containing a predetermined amount of Cu as well as the specific element, the high magnetic flux density  $B_8$  of 1.94 T or more was obtained. In Steel type MD1 and Steel type MD3 not containing the specific element, the low magnetic flux density  $B_8$  of 1.90 T or less was obtained. As above, combining Cu and the specific element made it possible to obtain a grain-oriented electrical steel sheet having a high magnetic flux density.

As shown in FIG. 1, in Steel type MD4 and Steel type MD6 to Steel type MD10 each containing the specific element and Cu and in Steel type MD5 with the Cu content being relatively high, the primary coating film was peeled off after bending to expose the steel sheet, resulting in failure of the adhesion. In Steel type MD1 with the Cu content being small and not containing the specific element, in Steel type MD2 with the Cu content being small, and in Steel type MD3 not containing the specific element, the primary coating film was not peeled off even after bending and the adhesion was good. As above, in the case where the grain-oriented electrical steel sheet was manufactured using the slab containing the specific element and Cu, the grain-oriented electrical steel sheet having a high magnetic flux density was obtained, but its adhesion deteriorated.

65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
780  
781  
782  
783  
784  
785  
786  
787  
788  
789  
790  
791  
792  
793  
794  
795  
796  
797  
798  
799  
800  
801  
802  
803  
804  
805  
806  
807  
808  
809  
8010  
8011  
8012  
8013  
8014  
8015  
8016  
8017  
8018  
8019  
8020  
8021  
8022  
8023  
8024  
8025  
8026  
8027  
8028  
8029  
8030  
8031  
8032  
8033  
8034  
8035  
8036  
8037  
8038  
8039  
8040  
8041  
8042  
8043  
8044  
8045  
8046  
8047  
8048  
8049  
8050  
8051  
8052  
8053  
8054  
8055  
8056  
8057  
8058  
8059  
8060  
8061  
8062  
8063  
8064  
8065  
8066  
8067  
8068  
8069  
8070  
8071  
8072  
8073  
8074  
8075  
8076  
8077  
8078  
8079  
8080  
8081  
8082  
8083  
8084  
8085  
8086  
8087  
8088  
8089  
8090  
8091  
8092  
8093  
8094  
8095  
8096  
8097  
8098  
8099  
80100  
80101  
80102  
80103  
80104  
80105  
80106  
80107  
80108  
80109  
80110  
80111  
80112  
80113  
80114  
80115  
80116  
80117  
80118  
80119  
80120  
80121  
80122  
80123  
80124  
80125  
80126  
80127  
80128  
80129  
80130  
80131  
80132  
80133  
80134  
80135  
80136  
80137  
80138  
80139  
80140  
80141  
80142  
80143  
80144  
80145  
80146  
80147  
80148  
80149  
80150  
80151  
80152  
80153  
80154  
80155  
80156  
80157  
80158  
80159  
80160  
80161  
80162  
80163  
80164  
80165  
80166  
80167  
80168  
80169  
80170  
80171  
80172  
80173  
80174  
80175  
80176  
80177  
80178  
80179  
80180  
80181  
80182  
80183  
80184  
80185  
80186  
80187  
80188  
80189  
80190  
80191  
80192  
80193  
80194  
80195  
80196  
80197  
80198  
80199  
80200  
80201  
80202  
80203  
80204  
80205  
80206  
80207  
80208  
80209  
80210  
80211  
80212  
80213  
80214  
80215  
80216  
80217  
80218  
80219  
80220  
80221  
80222  
80223  
80224  
80225  
80226  
80227  
80228  
80229  
80230  
80231  
80232  
80233  
80234  
80235  
80236  
80237  
80238  
80239  
80240  
80241  
80242  
80243  
80244  
80245  
80246  
80247  
80248  
80249  
80250  
80251  
80252  
80253  
80254  
80255  
80256  
80257  
80258  
80259  
80260  
80261  
80262  
80263  
80264  
80265  
80266  
80267  
80268  
80269  
80270  
80271  
80272  
80273  
80274  
80275  
80276  
80277  
80278  
80279  
80280  
80281  
80282  
80283  
80284  
80285  
80286  
80287  
80288  
80289  
80290  
80291  
80292  
80293  
80294  
80295  
80296  
80297  
80298  
80299  
80300  
80301  
80302  
80303  
80304  
80305  
80306  
80307  
80308  
80309  
80310  
80311  
80312  
80313  
80314  
80315  
80316  
80317  
80318  
80319  
80320  
80321  
80322  
80323  
80324  
80325  
80326  
80327  
80328  
80329  
80330  
80331  
80332  
80333  
80334  
80335  
80336  
80337  
80338  
80339  
80340  
80341  
80342  
80343  
80344  
80345  
80346  
80347  
80348  
80349  
80350  
80351  
80352  
80353  
80354  
80355  
80356  
80357  
80358  
80359  
80360  
80361  
80362  
80363  
80364  
80365  
80366  
80367  
80368  
80369  
80370  
80371  
80372  
80373  
80374  
80375  
80376  
80377  
80378  
80379  
80380  
80381  
80382  
80383  
80384  
80385  
80386  
80387  
80388  
80389  
80390  
80391  
80392  
80393  
80394  
80395  
80396  
80397  
80398  
80399  
80400  
80401  
80402  
80403  
80404  
80405  
80406  
80407  
80408  
80409  
80410  
80411  
80412  
80413  
80414  
80415  
80416  
80417  
80418  
80419  
80420  
80421  
80422  
80423  
80424  
80425  
80426  
80427  
80428  
80429  
80430  
80431  
80432  
80433  
80434  
80435  
80436  
80437  
80438  
80439  
80440  
80441  
80442  
80443  
80444  
80445  
80446  
80447  
80448  
80449  
80450  
80451  
80452  
80453  
80454  
80455  
80456  
80457  
80458  
80459  
80460  
80461  
80462  
80463  
80464  
80465  
80466  
80467  
80468  
80469  
80470  
80471  
80472  
80473  
80474  
80475  
80476  
80477  
80478  
80479  
80480  
80481  
80482  
80483  
80484  
80485  
80486  
80487  
80488  
80489  
80490  
80491  
80492  
80493  
80494  
80495  
80496  
80497  
80498  
80499  
80500  
80501  
80502  
80503  
80504  
80505  
80506  
80507  
80508  
80509  
80510  
80511  
80512  
80513  
80514  
80515  
80516  
80517  
80518  
80519  
80520  
80521  
80522  
80523  
80524  
80525  
80526  
80527  
80528  
80529  
80530  
80531  
80532  
80533  
80534  
80535  
80536  
80537  
80538  
80539  
80540  
80541  
80542  
80543  
80544  
80545  
80546  
80547  
80548  
80549  
80550  
80551  
80552  
80553  
80554  
80555  
80556  
80557  
80558  
80559  
80560  
80561  
80562  
80563  
80564  
80565  
80566  
80567  
80568  
80569  
80570  
80571  
80572  
80573  
80574  
80575  
80576  
80577  
80578  
80579  
80580  
80581  
80582  
80583  
80584  
80585  
80586  
80587  
80588  
80589  
80590  
80591  
80592  
80593  
80594  
80595  
80596  
80597  
80598  
8059

of slab heating before hot rolling. The Cu concentrated portion is extended by hot rolling, but is not dissolved in a hydrochloric acid or sulfuric acid aqueous solution, which is used for a general pickling bath, even in pickling after hot rolling. Therefore, it was considered that the Cu concentrated portion remains on the surface of the steel sheet even after cold rolling to impair the adhesion between the primary coating film and the steel sheet. As a result that in order to confirm this consideration, regarding Steel type MD4, the hot-rolled steel sheets resulting from hot rolling were subjected to pickling under various conditions to fabricate grain-oriented electrical steel sheets and the grain-oriented electrical steel sheets were subjected to the bending test similar to the above, the adhesion between the primary coating film and the steel sheet improved in the case where the pickling was performed under a specific condition.

Thus, the present inventors examined the effect of the Cu concentration at an interface region between the primary coating film and the steel sheet on the adhesion of the primary coating film. With Steel type MD3 and Steel type MD4, grain-oriented electrical steel sheets with different degrees of removing the Cu concentrated portion on the surface of the steel sheet were fabricated by variously changing the pickling condition after hot rolling, and each Cu concentration at an interface region between the primary coating film and the steel sheet was measured by GDS analysis (glow discharge optical emission spectrometry). Further, they examined the relationship between the Cu concentration at the interface region between the primary coating film and the steel sheet and the minimum bend radius at which peeling occurs while changing the bend radius to 10 mm to 30 mm. The peeling was defined as an area ratio of a peeled portion being 10% or more. Incidentally, a ratio of a Cu light-emitting intensity to an Fe light-emitting intensity in the GDS analysis, namely a Cu/Fe light-emitting intensity ratio was substituted for the Cu concentration. This is because the Cu concentration correlates with the Cu/Fe light-emitting intensity ratio. These results are illustrated in FIG. 2. As illustrated in FIG. 2, in Steel type MD3 not containing Te, the adhesion was good in each case and there was no correlation between the Cu concentration at the interface region between the primary coating film and the steel sheet and the adhesion. On the other hand, in Steel type MD4 containing Te, the adhesion was good in the case of the Cu concentration at the interface region between the primary coating film and the steel sheet being low (the Cu/Fe light-emitting intensity ratio being 0.30 or less).

In the case where Cu and the specific element such as Te coexist in the steel, when an oxide film containing an internal oxide  $\text{SiO}_2$  generated by decarburization annealing reacts with  $\text{MgO}$  in the annealing separating agent at the time of finish annealing, Cu and the specific element such as Te concentrated on the surface of the steel sheet together segregate to the interface between the steel sheet and the oxide film to form a liquid phase film. It is inferred that the adhesion of the primary coating film deteriorates because this liquid phase film suppresses the reaction of the oxide film containing the internal oxide  $\text{SiO}_2$  with  $\text{MgO}$  to planarize the structure of the interface between the primary coating film and the steel sheet.

Accordingly, it is conceived that as long as a steel sheet with a reduced Cu concentration on the surface of the steel sheet is used as the steel sheet before being subjected to the annealing separating agent application in the case of manufacture of the grain-oriented electrical steel sheet using the silicon steel material containing a specific element and Cu,

it is possible to manufacture a grain-oriented electrical steel sheet with a low Cu concentration at an interface region between a primary coating film and the steel sheet, and obtain a high magnetic flux density and excellent adhesion of the primary coating film.

The present invention has been made as a result of the above examinations. Hereinafter, there will be explained a grain-oriented electrical steel sheet, a decarburized steel sheet for the grain-oriented electrical steel sheet, and so on according to embodiments of the present invention.

There will be explained chemical compositions of the decarburized steel sheet for a grain-oriented electrical steel sheet according to the embodiment of the present invention and a slab used for its manufacture. Although their details will be described later, the decarburized steel sheet for a grain-oriented electrical steel sheet according to the embodiment of the present invention is manufactured by going through slab heating, hot rolling, hot-rolled sheet annealing, cold rolling, decarburization annealing, and so on. Thus, the chemical compositions of the decarburized steel sheet for a grain-oriented electrical steel sheet and the slab used for its manufacture consider not only properties of the decarburized steel sheet, but also these treatments. In the following explanation, being the unit of the content of each element contained in the decarburized steel sheet for a grain-oriented electrical steel sheet or the slab means "mass %" unless otherwise noted. The decarburized steel sheet for a grain-oriented electrical steel sheet according to this embodiment includes a chemical composition represented by C: 0.03% to 0.15%, Si: 1.8% to 7.0%, Mn: 0.02% to 0.30%, S: 0.005% to 0.040%, acid-soluble Al: 0.010% to 0.065%, N: 0.0030% to 0.0150%, Cu: 0.03% to 0.60%, Sn: 0% to 0.5%, Ge, Se, Sb, Te, Pb, or Bi, or an arbitrary combination of these: 0.0005% to 0.030% in total, and the balance: Fe and impurities. Examples of the impurities include ones contained in raw materials such as ore and scrap and ones contained in manufacturing steps.

(C: 0.03% to 0.15%)

C stabilizes secondary recrystallization. When the C content is less than 0.03%, crystal grains grow abnormally at the time of slab heating, and the secondary recrystallization becomes insufficient in finish annealing when manufacturing the grain-oriented electrical steel sheet. Thus, the C content is set to 0.03% or more. When the C content is greater than 0.15%, the time taken for decarburization annealing after cold rolling is prolonged and further decarburization becomes likely to be insufficient, so that magnetic aging is caused in a product. Thus, the C content is set to 0.15% or less.

(Si: 1.8% to 7.0%)

Si increases an electrical resistance of steel to reduce an eddy current loss. When the Si content is less than 1.8%, it is impossible to suppress the eddy current loss of the product. Thus, the Si content is set to 1.8% or more. When the Si content is greater than 7.0%, workability deteriorates significantly, to thus make it difficult to perform cold rolling at normal temperature. Thus, the Si content is set to 7.0% or less.

(Mn: 0.02% to 0.30%)

Mn forms MnS functioning as an inhibitor. When the Mn content is less than 0.02%, MnS necessary for causing the secondary recrystallization falls short. Thus, the Mn content is set to 0.02% or more. When the Mn content is greater than 0.30%, it becomes difficult to solid-dissolve MnS at the time of slab heating, and further the size of MnS to precipitate again at the time of hot rolling becomes likely to be coarse. Thus, the Mn content is set to 0.30% or less.

(S: 0.005% to 0.040%)

S forms MnS functioning as an inhibitor with Mn. When the S content is less than 0.005%, it is impossible to obtain an inhibitor effect sufficient for exhibiting the secondary recrystallization. Thus, the S content is set to 0.005% or more. When the S content is greater than 0.040%, edge cracking becomes likely to occur at the time of hot rolling. Thus, the S content is set to 0.040% or less.

(Acid-Soluble Al: 0.010% to 0.065%)

Al forms AlN functioning as an inhibitor. When the Al content is less than 0.010%, AlN falls short and an inhibitor strength is low, and thus an effect of the above is not exhibited. Thus, the Al content is set to 0.010% or more. When the Al content is greater than 0.065%, AlN becomes coarse to reduce the inhibitor strength. Thus, the Al content is set to 0.065% or less.

(N: 0.0030% to 0.0150%)

N forms AlN functioning as an inhibitor with Al. When the N content is less than 0.0030%, it is impossible to obtain a sufficient inhibitor effect. Thus, the N content is set to 0.0030% or more. When the N content is greater than 0.0150%, surface flaws called blisters occur. Thus, the N content is set to 0.0150% or less.

(Cu: 0.03% to 0.60%)

Cu remains in the steel sheet to increase a specific resistance of the steel sheet and reduce a core loss. Further, Cu strengthens the inhibitors necessary for the secondary recrystallization and increases a magnetic flux density of the grain-oriented electrical steel sheet. When the Cu content is less than 0.03%, it is impossible to sufficiently obtain a function effect of the above and stably manufacture a grain-oriented electrical steel sheet having a high magnetic flux density. Thus, the Cu content is set to 0.03% or more. When the Cu content is greater than 0.60%, the function effect is saturated. Thus, the Cu content is set to 0.60% or less.

(Ge, Se, Sb, Te, Pb, or Bi, or an arbitrary combination of these: 0.0005% to 0.030% in total)

Ge, Se, Sb, Te, Pb, and Bi strengthen the inhibitors, improve the magnetic flux density, and contribute to stable manufacture of a grain-oriented electrical steel sheet having a magnetic flux density  $B_g$  of 1.94 T or more. When Ge, Se, Sb, Te, Pb, or Bi, or an arbitrary combination of these is less than 0.0005% in total, an effect of the above is small. Thus, Ge, Se, Sb, Te, Pb, or Bi, or an arbitrary combination of these is set to 0.0005% or more in total. When Ge, Se, Sb, Te, Pb, or Bi, or an arbitrary combination of these is greater than 0.030% in total, coating film adhesion deteriorates significantly as well as saturation of the effect. Thus, Ge, Se, Sb, Te, Pb, or Bi, or an arbitrary combination of these is set to 0.030% or less in total. Ge, Se, Sb, Te, Pb, and Bi each have a small solid solubility in iron, and are likely to aggregate at the interface between the primary coating film and the steel sheet, or at the interface between precipitates and the steel sheet. Such a property is effective for strengthening the inhibitors, but tends to adversely affect formation of the primary coating film, so that it is inferred that the property impairs the coating film adhesion.

Sn is not an essential element, but an arbitrary element that may be appropriately contained, up to a predetermined amount as a limit, in the decarburized steel sheet for a grain-oriented electrical steel sheet.

(Sn: 0% to 0.5%)

Sn stabilizes the secondary recrystallization and makes the diameter of secondary recrystallized grains small. Thus, Sn may be contained. The Sn content is preferably set to 0.05% or more in order to sufficiently obtain a function

effect of the above. When the Sn content is greater than 0.5%, the function effect is saturated. Thus, the Sn content is set to 0.5% or less. In order to more reduce occurrence of cracking during cold rolling to thereby more increase a yield of the product, the Sn content is preferably set to 0.2% or less.

The decarburized steel sheet for a grain-oriented electrical steel sheet according to the embodiment of the present invention includes an oxide film on the surface of the steel sheet, and a Cu/Fe light-emitting intensity ratio at an interface region between the oxide film and the surface of the steel sheet is 0.60 or less. The Cu/Fe light-emitting intensity ratio at the interface region between the oxide film formed by decarburization annealing and the surface of the steel sheet is 0.60 or less, thereby preventing an increase in Cu concentration at an interface region between the primary coating film to be formed thereafter and the steel sheet. For obtaining higher adhesion between the primary coating film and the steel sheet, the Cu/Fe light-emitting intensity ratio at the interface region between the oxide film and the surface of the steel sheet is preferably 0.40 or less.

The Cu/Fe light-emitting intensity ratio obtained by using the GDS analysis is substituted for the Cu concentration at the interface region between the oxide film in the decarburized steel sheet and the steel sheet. This is because the Cu concentration correlates with the Cu/Fe light-emitting intensity ratio. The interface region means the following region. Measurement of element distributions in a depth direction by the GDS analysis reveals that the peak strengths of O and Si, which are the main elements forming the oxide film, decrease from the surface of the decarburized steel sheet to the inside, while the peak strength of Fe increases. The interface region is a region ranging between the depth from the surface of the decarburized steel sheet that corresponds to the sputtering time when the peak strength of Fe becomes maximum and the depth from the surface of the decarburized steel sheet that corresponds to the sputtering time when the peak strength of Fe becomes  $\frac{1}{2}$  of the maximum peak strength. In the GDS analysis, detection wavelengths used when measuring the Cu light-emitting intensity and the Fe light-emitting intensity are set to 327.396 nm and 271.903 nm respectively. Measurement examples of the Fe light-emitting intensity, the Cu light-emitting intensity, and the Cu/Fe light-emitting intensity ratio, which are obtained by using the GDS analysis, are illustrated in FIG. 3. A region A in FIG. 3 is the interface region specified as above. The Cu/Fe light-emitting intensity ratio is evaluated by the “average of (Cu light-emitting intensities/Fe light-emitting intensities) at respective measurement points in the interface region” at the interface region specified as above.

Next, the chemical composition of the grain-oriented electrical steel sheet according to the embodiment of the present invention will be explained. Although its detail will be described later, the grain-oriented electrical steel sheet according to the embodiment of the present invention is manufactured by going through slab heating, hot rolling, hot-rolled sheet annealing, cold rolling, annealing separating agent application, finish annealing, and so on. Purification annealing may be included in the finish annealing. Thus, the chemical composition of the grain-oriented electrical steel sheet considers not only properties of the grain-oriented electrical steel sheet, but also these treatments. In the following explanation, “%” being the unit of the content of each element contained in the grain-oriented electrical steel sheet means “mass %” unless otherwise noted. The grain-oriented electrical steel sheet according to this embodiment includes a chemical composition represented by Si: 1.8% to

## 11

7.0%, Cu: 0.03% to 0.60%, and the balance: Fe and impurities. Examples of the impurities include ones contained in raw materials such as ore and scrap and ones contained in manufacturing steps, and concretely, Mn, Al, C, N, S, and so on are taken as an example. Further, an element such as B derived from the annealing separating agent may remain as an impurity.

(Si: 1.8% to 7.0%)

Si increases an electrical resistance of steel to reduce an eddy current loss. When the Si content is less than 1.8%, it is impossible to obtain a function effect of the above. Thus, the Si content is set to 1.8% or more. When the Si content is greater than 7.0%, workability deteriorates significantly. Thus, the Si content is set to 7.0% or less.

(Cu: 0.03% to 0.60%)

Cu strengthens the function of inhibitors at the time of manufacture of the grain-oriented electrical steel sheet and highly accumulates crystal grain orientations of a product in the {110}<001> orientation, and containing Cu with a specific element further increases an effect of the above. Further, even when remaining finally, Cu increases a specific resistance to reduce a core loss. When the Cu content is less than 0.03%, it is impossible to sufficiently obtain a function effect of the above. Thus, the Cu content is set to 0.03% or more. When the Cu content is greater than 0.60%, the function effect is saturated. Thus, the Cu content is set to 0.60% or less. Incidentally, in the case where scrap is mixed as a raw material when melting the steel, Cu may be mixed in from the scrap.

The grain-oriented electrical steel sheet according to the embodiment of the present invention includes a primary coating film containing forsterite on the surface of the steel sheet, and a Cu/Fe light-emitting intensity ratio at an interface region between the primary coating film and the surface of the steel sheet is 0.30 or less. Forsterite, which is the main component out of components composing the primary coating film, is contained by 70 mass % or more. The Cu/Fe light-emitting intensity ratio is 0.30 or less, thereby making it possible to obtain a grain-oriented electrical steel sheet excellent in adhesion between the primary coating film and the steel sheet. For obtaining higher adhesion between the primary coating film and the steel sheet, the Cu/Fe light-emitting intensity ratio at the interface region between the primary coating film and the surface of the steel sheet is preferably 0.20 or less.

The Cu/Fe light-emitting intensity ratio obtained by using the GDS analysis is substituted for the Cu concentration at the interface region between the primary coating film in the grain-oriented electrical steel sheet and the steel sheet. This is because the Cu concentration correlates with the Cu/Fe light-emitting intensity ratio. The interface region means the following region. Measurement of element distributions in the depth direction by the GDS analysis reveals that the peak strengths of O, Mg, and Si, which are the main elements forming the primary coating film, decrease from the surface of the grain-oriented electrical steel sheet to the inside, while the peak strength of Fe increases. The interface region is a region ranging between the depth from the surface of the grain-oriented electrical steel sheet that corresponds to the sputtering time when the peak strength of Fe becomes maximum and the depth from the surface of the grain-oriented electrical steel sheet that corresponds to the sputtering time when the peak strength of Fe becomes  $\frac{1}{2}$  of the maximum peak strength. Incidentally, the depth from the surface of the grain-oriented electrical steel sheet corresponding to the sputtering time when the peak strength of Fe becomes maximum is also substantially equivalent to the

## 12

depth where the peak strength of Mg is no longer detected. In the GDS analysis, detection wavelengths used when measuring the Cu light-emitting intensity and the Fe light-emitting intensity are set to 327.396 nm and 271.903 nm respectively.

Next, there will be explained a manufacturing method of the decarburized steel sheet for a grain-oriented electrical steel sheet according to the embodiment of the present invention. In the manufacturing method of the decarburized steel sheet for a grain-oriented electrical steel sheet according to this embodiment, there are performed slab heating, hot rolling, hot-rolled sheet annealing, cold rolling, decarbonization annealing, pickling, and so on.

First, a molten steel used for manufacture of the above-described decarburized steel sheet is formed into a slab by an ordinary method, and then the slab is heated and subjected to hot rolling.

When the slab heating temperature is less than 1300°C., it is impossible to melt precipitates such as MnS, so that the variation in magnetic flux density of the product is large. Thus, the slab heating temperature is set to 1300°C. or more. When the slab heating temperature is greater than 1490°C., the slab melts. Thus, the slab heating temperature is set to 1490°C. or less.

In the hot rolling, rough rolling with a finishing temperature set to 1200°C. or less is performed, and finish rolling with a start temperature set to 1000°C. or more and a finishing temperature set to 950°C. to 1100°C. is performed. When the finishing temperature of the rough rolling is greater than 1200°C., precipitation of MnS or MnSe in the rough rolling is not promoted, resulting in that Cu<sub>2</sub>S is generated in the finish rolling and the magnetic property of the product deteriorates. Thus, the finishing temperature of the rough rolling is set to 1200°C. or less. When the start temperature of the finish rolling is less than 1000°C., the finishing temperature of the finish rolling falls below 950°C., resulting in that Cu<sub>2</sub>S becomes likely to precipitate and the magnetic property of the product does not stabilize. Thus, the start temperature of the finish rolling is set to 1000°C. or more. When the finishing temperature of the finish rolling is less than 950°C., Cu<sub>2</sub>S becomes likely to precipitate and the magnetic property does not stabilize. Further, when the difference in temperature from the slab heating temperature is too large, it is difficult to make temperature histories over the entire length of a hot-rolled coil uniform, and thus it becomes difficult to form homogeneous inhibitors over the entire length of the hot-rolled coil. Thus, the finishing temperature of the finish rolling is set to 950°C. or more. When the finishing temperature of the finish rolling is greater than 1100°C., it is impossible to control fine dispersion of MnS and MnSe. Thus, the finishing temperature of the finish rolling is set to 1100°C. or less.

The finish rolling is started within 300 seconds after start of the rough rolling. When the time period between start of the rough rolling and start of the finish rolling is greater than 300 seconds, MnS or MnSe having 50 nm or less, which functions as an inhibitor, is no longer dispersed, grain diameter control in decarbonization annealing and secondary recrystallization in finish annealing become difficult, and the magnetic property deteriorates. Thus, the time period between start of the rough rolling and start of the finish rolling is set to within 300 seconds. Incidentally, the lower limit of the time period does not need to be set in particular as long as the rolling is normal rolling. When the time period between start of the rough rolling and start of the finish rolling is less than 30 seconds, a precipitation amount of

MnS or MnSe is not sufficient and secondary recrystallized crystal grains become difficult to grow at the time of finish annealing in some cases.

Cooling at a cooling rate of 50° C./second or more is started within 10 seconds after finish of the finish rolling. When the time period between finish of the finish rolling and start of the cooling is greater than 10 seconds, Cu<sub>2</sub>S becomes likely to precipitate and the magnetic property of the product does not stabilize. Thus, the time period between finish of the finish rolling and start of the cooling is set to within 10 seconds, and preferably set to within two seconds. When the cooling rate after the finish rolling is less than 50° C./second, Cu<sub>2</sub>S becomes likely to precipitate and the magnetic property of the product does not stabilize. Thus, the cooling rate after the finish rolling is set to 50° C./second or more.

Thereafter, coiling is performed in a temperature zone of 600° C. or less. When the coiling temperature is greater than 600° C., Cu<sub>2</sub>S becomes likely to precipitate and the magnetic property of the product does not stabilize. Thus, the coiling temperature is set to 600° C. or less.

Next, hot-rolled sheet annealing of an obtained hot-rolled steel sheet is performed. When the finishing temperature of the finish rolling is set to Tf, the holding temperature of the hot-rolled sheet annealing is set to 950° C. to (Tf+100° C.). When the holding temperature is less than 950° C., it is impossible to make the inhibitors homogeneous over the entire length of the hot-rolled coil and the magnetic property of the product does not stabilize. Thus, the holding temperature is set to 950° C. or more. When the holding temperature is greater than (Tf+100° C.), MnS that has finely precipitated in the hot rolling grows rapidly and the secondary recrystallization is destabilized. Thus, the holding temperature is set to (Tf+100°) C. or less.

Next, one cold rolling, or two or more cold rollings with intermediate annealing therebetween are performed to obtain a cold-rolled steel sheet. Thereafter, decarburization annealing of the cold-rolled steel sheet is performed. By performing the decarburization annealing, an oxide film containing SiO<sub>2</sub> is formed on the surface of the steel sheet. The cold rolling and the decarburization annealing can be performed by general methods.

After the hot rolling and before finish of the cold rolling, for example, between the hot rolling and the hot-rolled sheet annealing, or between the hot-rolled sheet annealing and the cold rolling, pickling with a holding temperature set to 50° C. or more and a holding time period set to 30 seconds or more is performed in a pickling bath containing a nitric acid, a pickling inhibitor, and a surface active agent. Performing such pickling enables a Cu concentrated portion on the surface of the steel sheet to be removed. Removing the Cu concentrated portion enables the Cu/Fe light-emitting intensity ratio obtained by the GDS analysis to be 0.60 or less in terms of the Cu concentration on the surface of the decarburized steel sheet resulting from the decarburization annealing. When the content of the nitric acid is less than 5 g/l, it is impossible to sufficiently remove the Cu concentrated portion. Thus, the content of the nitric acid is set to 5 g/l or more. When the content of the nitric acid is greater than 200 g/l, its function effect is saturated and its cost increases. Thus, the content of the nitric acid is set to 200 g/l or less. When the content of the pickling inhibitor is less than 0.5 g/l, excessive dissolution of the surface of the steel sheet occurs locally to make the surface uneven and extremely rough. Thus, the content of the pickling inhibitor is set to 0.5 g/l or more. When the content of the pickling inhibitor is greater than 10 g/l, its function effect is saturated and its cost increases. Thus, the content of the pickling inhibitor is set to

10 g/l or less. When the content of the surface active agent is less than 0.5 g/l, it is impossible to sufficiently remove the Cu concentrated portion. Thus, the content of the surface active agent is set to 0.5 g/l or more. When the content of the surface active agent is greater than 10 g/l, its function effect is saturated and its cost increases. Thus, the content of the surface active agent is set to 10 g/l or less. When the holding temperature is less than 50° C., the rate of removing scales by the pickling decreases significantly and the productivity decreases. Thus, the holding temperature is set to 50° C. or more. When the holding time period is less than 30 seconds, it is impossible to sufficiently remove scales. Thus, the holding time period is set to 30 seconds or more.

As the pickling inhibitor, it is possible to use an organic inhibitor preferably, and for example, an amine derivative, mercaptans, sulfides, thiourea and its derivative, or the like can be used. As the surface active agent, it is possible to use ethylene glycol, glycerin, or the like preferably.

The pickling bath may contain a nitrate, for example, sodium nitrate. The pickling is performed in the pickling bath containing a nitrate, thereby enabling more secure removal of the Cu concentrated portion on the surface of the steel sheet and enabling the Cu/Fe light-emitting intensity ratio obtained by the GDS analysis to be 0.40 or less in terms of the Cu concentration on the surface of the decarburized steel sheet resulting from the decarburization annealing. When the content of the nitrate is less than 0.5 g/l, it is sometimes impossible to securely remove the Cu concentrated portion. Thus, the content of the nitrate is set to 0.5 g/l or more. When the content of the nitrate is greater than 10 g/l, its function effect is saturated and its cost increases. Thus, the content of the nitrate is set to 10 g/l or less.

In this manner, it is possible to manufacture the decarburized steel sheet for a grain-oriented electrical steel sheet according to this embodiment.

Next, there will be explained a manufacturing method of the grain-oriented electrical steel sheet according to the embodiment of the present invention. In the manufacturing method of the grain-oriented electrical steel sheet according to this embodiment, there are performed slab heating, hot rolling, hot-rolled sheet annealing, cold rolling, decarburization annealing, annealing separating agent application, finish annealing, pickling, and so on. The slab heating, the hot rolling, the hot-rolled sheet annealing, the cold rolling, the decarburization annealing, and the pickling can be performed similarly to the above-described manufacturing method of the decarburized steel sheet for a grain-oriented electrical steel sheet.

The obtained decarburized steel sheet has an annealing separating agent containing MgO applied thereto to be subjected to finish annealing. Pickling is performed after hot rolling and before finish of cold rolling. The annealing separating agent contains MgO, and the ratio of MgO in the annealing separating agent is 90 mass % or more, for example. In the finish annealing, purification annealing may be performed after the secondary recrystallization is completed. The annealing separating agent application and the finish annealing can be performed by general methods.

The pickling is performed to control the Cu concentration on the surface of the steel sheet, and thereby the Cu/Fe light-emitting intensity ratio obtained by the GDS analysis becomes 0.30 or less, in terms of the Cu concentration at an interface region between a primary coating film mainly composed of forsterite formed on the surface of the steel sheet after finish annealing to be performed thereafter and the steel sheet. Further, the pickling is performed in a pickling bath containing a nitrate, thereby enabling more

secure removal of the Cu concentrated portion on the surface of the steel sheet and enabling the Cu/Fe light-emitting intensity ratio obtained by the GDS analysis to be 0.20 or less in terms of the Cu concentration at the interface region between the primary coating film formed on the surface of the steel sheet after the finish annealing and the steel sheet.

In this manner, it is possible to manufacture the grain-oriented electrical steel sheet according to this embodiment. After the finish annealing, an insulating coating film may be formed by application and baking.

From the above, according to the manufacturing method of the decarburized steel sheet for a grain-oriented electrical steel sheet and the manufacturing method of the grain-oriented electrical steel sheet according to the embodiments of the present invention, it is possible to appropriately control the Cu concentration on the surface of the steel sheet and obtain the grain-oriented electrical steel sheet having a good magnetic property and having excellent adhesion between the primary coating film and the steel sheet and the decarburized steel sheet for the grain-oriented electrical steel sheet.

In the foregoing, the preferred embodiments of the present invention have been described in detail, but, the present invention is not limited to such examples. It is apparent that a person having common knowledge in the technical field to which the present invention belongs is able to devise various variation or modification examples within the range of technical ideas described in the claims, and it should be understood that such examples belong to the technical scope of the present invention as a matter of course.

#### EXAMPLE

Next, the decarburized steel sheet for a grain-oriented electrical steel sheet and the grain-oriented electrical steel sheet according to the embodiments of the present invention will be explained concretely while referring to examples. The following examples are merely examples of the decarburized steel sheet for a grain-oriented electrical steel sheet and the grain-oriented electrical steel sheet according to the embodiments of the present invention, and the decarburized steel sheet for a grain-oriented electrical steel sheet and the grain-oriented electrical steel sheet according to the present invention are not limited to the following examples.

In a vacuum melting furnace, silicon steel materials having chemical compositions of Steel type MD4 to Steel type MD10 illustrated in Table 1 were fabricated, and after being heated at temperatures illustrated in Table 3 to Table 5, slabs were subjected to hot rolling under conditions

illustrated in Table 3 to Table 5 to obtain hot-rolled steel sheets having a sheet thickness of 2.3 mm, and they were coiled at temperatures illustrated in Table 3 to Table 5. Then, after being annealed, the hot-rolled steel sheets were subjected to pickling using a pickling bath B1 to a pickling bath B3 illustrated in Table 6. As a nitrate contained in the pickling bath B2, sodium nitrate was used. Thereafter, cold rolling was performed under conditions illustrated in Table 3 to Table 5, and cold-rolled steel sheets having a sheet thickness of 0.22 mm were obtained. Then, the obtained cold-rolled steel sheets were subjected to primary recrystallization annealing including decarburization annealing, to thereby obtain decarburized steel sheets, and then the decarburized steel sheets had an annealing separating agent containing MgO as its main component applied thereto and were subjected to finish annealing, and an insulating coating film was applied to obtained finish-annealed sheets to be baked to obtain grain-oriented electrical steel sheets.

Each sample was taken from the obtained decarburized steel sheets and grain-oriented electrical steel sheets to be subjected to GDS analysis, the Cu light-emitting intensity and the Fe light-emitting intensity at the interface region between the oxide film and the steel sheet were measured in each of the decarburized steel sheets, and the Cu light-emitting intensity and the Fe light-emitting intensity at the interface region between the primary coating film mainly composed of forsterite and the steel sheet were measured in each of the grain-oriented electrical steel sheets to obtain each Cu/Fe light-emitting intensity ratio. Each sample was taken from the obtained grain-oriented electrical steel sheets to measure each magnetic flux density  $B_g$ . Each sample was taken from a portion 50 mm apart from the end in the coil width direction in the finish annealing and from the center portion in the coil width direction, and they were each subjected to a bending test in which each sample was wound on a 20-mm  $\phi$  cylindrical body. The length of the portion deformed on a curved surface of the cylindrical body by this bending was about 30 mm, and each coating film adhesion was evaluated according to a coating film residual ratio in the deformed portion. As for the evaluation of the coating film adhesion, the case of the coating film residual ratio being 70% or more was judged to be excellent in coating film adhesion. These results are illustrated in Table 3 to Table 5. Incidentally, each underline in Table 3 to Table 5 indicates that a corresponding numerical value is outside the range of the present invention. Each underline in Table 6 indicates that a corresponding condition is outside the range of the present invention.

TABLE 3

| SAMPLE<br>No. | STEEL<br>TYPE | SLAB HEATING<br>TEMPERATURE<br>(° C.) | ROUGH<br>ROLLING                   |                             | STANDBY<br>TIME<br>(SECOND) | START<br>TEMPERATURE<br>(° C.) | FINISHING<br>TEMPERATURE<br>(° C.) | STANDBY<br>TIME<br>(SECOND) | COOLING<br>RATE<br>(° C./SECOND) |
|---------------|---------------|---------------------------------------|------------------------------------|-----------------------------|-----------------------------|--------------------------------|------------------------------------|-----------------------------|----------------------------------|
|               |               |                                       | FINISHING<br>TEMPERATURE<br>(° C.) | STANDBY<br>TIME<br>(SECOND) |                             |                                |                                    |                             |                                  |
| 1             | MD4           | 1350                                  | 1150                               | 60                          |                             | 1100                           | 1060                               | 1.2                         | 80                               |
| 2             | MD4           | 1350                                  | 1150                               | 60                          |                             | 1100                           | 1060                               | 1.2                         | 80                               |
| 3             | MD4           | 1350                                  | 1150                               | 60                          |                             | 1100                           | 1060                               | 1.2                         | 80                               |
| 4             | MD4           | 1280                                  | 1110                               | 30                          |                             | 1080                           | 1050                               | 1                           | 80                               |
| 5             | MD4           | 1500                                  |                                    |                             |                             |                                |                                    |                             |                                  |
| 6             | MD4           | 1350                                  | 1220                               | 80                          |                             | 1100                           | 1050                               | 1                           | 80                               |
| 7             | MD4           | 1350                                  | 1150                               | 320                         |                             | 1100                           | 1050                               | 1                           | 80                               |
| 8             | MD4           | 1350                                  | 1150                               | 110                         |                             | 980                            | 1000                               | 1                           | 80                               |
| 9             | MD4           | 1350                                  | 1150                               | 60                          |                             | 1100                           | 930                                | 1                           | 60                               |

HOT ROLLING IMPOSSIBLE

TABLE 3-continued

|    |            |             |             |            |            |             |           |           |
|----|------------|-------------|-------------|------------|------------|-------------|-----------|-----------|
| 10 | MD4        | 1350        | 1150        | 10         | 1130       | <u>1120</u> | 1         | 90        |
| 11 | MD4        | 1350        | 1150        | 60         | 1100       | 1060        | <u>12</u> | 80        |
| 12 | MD4        | 1350        | 1150        | 60         | 1100       | 1060        | 1.2       | <u>45</u> |
| 13 | MD4        | 1350        | 1150        | 60         | 1100       | 1060        | 1.2       | 80        |
| 14 | <u>MD5</u> | 1350        | 1150        | 60         | 1100       | 1060        | 1.2       | 80        |
| 15 | <u>MD5</u> | 1350        | 1150        | 60         | 1100       | 1060        | 1.2       | 80        |
| 16 | <u>MD5</u> |             | 1150        | 60         | 1100       | 1060        | 1.2       | 80        |
| 17 | <u>MD5</u> | <u>1280</u> | 1110        | 30         | 1080       | 1050        | 1         | 80        |
| 18 | <u>MD5</u> | <u>1500</u> |             |            |            |             |           |           |
| 19 | <u>MD5</u> | 1350        | <u>1220</u> | 80         | 1100       | 1050        | 1         | 80        |
| 20 | <u>MD5</u> | 1350        | 1150        | <u>320</u> | 1100       | 1050        | 1         | 80        |
| 21 | <u>MD5</u> | 1350        | 1150        | <u>110</u> | <u>980</u> | 1000        | 1         | 80        |
| 22 | <u>MD5</u> | 1350        | 1150        | 60         | 1100       | <u>930</u>  | 1         | 60        |
| 23 | <u>MD5</u> | 1350        | 1150        | 10         | 1130       | <u>1120</u> | 1         | 90        |
| 24 | <u>MD5</u> | 1350        | 1150        | 60         | 1100       | 1060        | <u>12</u> | 80        |
| 25 | <u>MD5</u> | 1350        | 1150        | 60         | 1100       | 1060        | 1.2       | <u>45</u> |
| 26 | <u>MD5</u> | 1350        | 1150        | 60         | 1100       | 1060        | 1.2       | 80        |
| 27 | MD6        | 1350        | 1150        | 60         | 1100       | 1060        | 1.2       | 80        |
| 28 | MD6        | 1350        | 1150        | 60         | 1100       | 1060        | 1.2       | 80        |
| 29 | MD6        | 1350        | 1150        | 60         | 1100       | 1060        | 1.2       | 80        |
| 30 | MD6        | <u>1280</u> | 1110        | 30         | 1080       | 1050        | 1         | 80        |

# GRAIN-ORIENTED ELECTRICAL STEEL SHEET

| SAMPLE<br>No. | COILING<br>TEMPERATURE<br>(° C.) | PICKLING<br>BATH<br>TYPE | STEEL SHEET<br>LIGHT-<br>EMMITING<br>INTENSITY<br>RATIO | LIGHT-<br>EMMITING<br>INTENSITY<br>RATIO | MAGNETIC<br>FLUX<br>DENSITY B <sub>8</sub><br>(T) | COATING<br>FILM<br>RESIDUAL<br>RATIO<br>(%) |  |
|---------------|----------------------------------|--------------------------|---------------------------------------------------------|------------------------------------------|---------------------------------------------------|---------------------------------------------|--|
|               |                                  |                          |                                                         |                                          |                                                   |                                             |  |
| 1             | 550                              | B1                       | 0.52                                                    | 0.28                                     | 1.94                                              | 95                                          |  |
| 2             | 550                              | B2                       | 0.40                                                    | 0.15                                     | 1.94                                              | 100                                         |  |
| 3             | 550                              | <u>B3</u>                | 0.65                                                    | <u>0.41</u>                              | 1.94                                              | 50                                          |  |
| 4             | 550                              | B2                       | 0.41                                                    | 0.17                                     | 1.82                                              | 100                                         |  |
| 5             | HOT ROLLING<br>IMPOSSIBLE        | B2                       |                                                         |                                          | MEASUREMENT IMPOSSIBLE                            |                                             |  |
| 6             | 550                              | B2                       | 0.40                                                    | 0.15                                     | 1.88                                              | 100                                         |  |
| 7             | 550                              | B2                       | 0.40                                                    | 0.15                                     | 1.83                                              | 100                                         |  |
| 8             | 550                              | B2                       | 0.40                                                    | 0.15                                     | 1.86                                              | 100                                         |  |
| 9             | 550                              | B2                       | 0.40                                                    | 0.15                                     | 1.89                                              | 100                                         |  |
| 10            | 550                              | B2                       | 0.40                                                    | 0.15                                     | 1.83                                              | 100                                         |  |
| 11            | 550                              | B2                       | 0.40                                                    | 0.16                                     | 1.88                                              | 100                                         |  |
| 12            | 550                              | B2                       | 0.40                                                    | 0.15                                     | 1.89                                              | 100                                         |  |
| 13            | <u>620</u>                       | B2                       | 0.40                                                    | 0.16                                     | 1.92                                              | 100                                         |  |
| 14            | 550                              | B1                       | <u>0.80</u>                                             | <u>0.60</u>                              | 1.90                                              | 50                                          |  |
| 15            | 550                              | B2                       | <u>0.70</u>                                             | <u>0.50</u>                              | 1.91                                              | 50                                          |  |
| 16            | 550                              | <u>B3</u>                | <u>1.10</u>                                             | <u>0.80</u>                              | 1.90                                              | 40                                          |  |
| 17            | 550                              | B2                       | <u>0.72</u>                                             | <u>0.55</u>                              | 1.90                                              | 40                                          |  |
| 18            | HOT ROLLING<br>IMPOSSIBLE        | B2                       |                                                         |                                          | MEASUREMENT IMPOSSIBLE                            |                                             |  |
| 19            | 550                              | B2                       | <u>0.72</u>                                             | <u>0.52</u>                              | 1.88                                              | 50                                          |  |
| 20            | 550                              | B2                       | <u>0.72</u>                                             | <u>0.52</u>                              | 1.85                                              | 50                                          |  |
| 21            | 550                              | B2                       | <u>0.72</u>                                             | <u>0.50</u>                              | 1.90                                              | 30                                          |  |
| 22            | 550                              | B2                       | <u>0.72</u>                                             | <u>0.52</u>                              | 1.90                                              | 30                                          |  |
| 23            | 550                              | B2                       | <u>0.72</u>                                             | <u>0.52</u>                              | 1.86                                              | 50                                          |  |
| 24            | 550                              | B2                       | <u>0.72</u>                                             | <u>0.52</u>                              | 1.91                                              | 30                                          |  |
| 25            | 550                              | B2                       | <u>0.72</u>                                             | <u>0.55</u>                              | 1.90                                              | 50                                          |  |
| 26            | <u>620</u>                       | B2                       | <u>0.72</u>                                             | <u>0.55</u>                              | 1.88                                              | 40                                          |  |
| 27            | 550                              | B1                       | 0.25                                                    | 0.18                                     | 1.94                                              | 90                                          |  |
| 28            | 550                              | B2                       | 0.20                                                    | 0.10                                     | 1.94                                              | 100                                         |  |
| 29            | 550                              | <u>B3</u>                | 0.40                                                    | <u>0.35</u>                              | 1.94                                              | 70                                          |  |
| 30            | 550                              | B2                       | 0.40                                                    | <u>0.35</u>                              | 1.94                                              | 95                                          |  |

TABLE 4

## HOT ROLLING

| SAMPLE<br>No. | STEEL<br>TYPE | SLAB HEATING<br>TEMPERATURE<br>(° C.) | ROUGH<br>ROLLING                   |                             | FINISH<br>ROLLING | FINISH<br>ROLLING      | COOLING                     |                                  |
|---------------|---------------|---------------------------------------|------------------------------------|-----------------------------|-------------------|------------------------|-----------------------------|----------------------------------|
|               |               |                                       | FINISHING<br>TEMPERATURE<br>(° C.) | STANDBY<br>TIME<br>(SECOND) |                   |                        | STANDBY<br>TIME<br>(SECOND) | COOLING<br>RATE<br>(° C./SECOND) |
| 31            | MD6           | 1500                                  |                                    |                             |                   | HOT ROLLING IMPOSSIBLE |                             |                                  |
| 32            | MD6           | 1350                                  | 1220                               | 80                          | 1100              | 1050                   | 1                           | 80                               |

TABLE 4-continued

|    |     |             |             |            |            |                        |           |           |
|----|-----|-------------|-------------|------------|------------|------------------------|-----------|-----------|
| 33 | MD6 | 1350        | 1150        | <u>320</u> | 1100       | 1050                   | 1         | 80        |
| 34 | MD6 | 1350        | 1150        | 110        | <u>980</u> | 1000                   | 1         | 80        |
| 35 | MD6 | 1350        | 1150        | 60         | 1100       | <u>930</u>             | 1         | 60        |
| 36 | MD6 | 1350        | 1150        | 10         | 1130       | <u>1120</u>            | 1         | 90        |
| 37 | MD6 | 1350        | 1150        | 60         | 1100       | 1060                   | <u>12</u> | 80        |
| 38 | MD6 | 1350        | 1150        | 60         | 1100       | 1060                   | 1.2       | <u>45</u> |
| 39 | MD6 | 1350        | 1150        | 60         | 1100       | 1060                   | 1.2       | 80        |
| 40 | MD7 | 1350        | 1150        | 60         | 1100       | 1060                   | 1.2       | 80        |
| 41 | MD7 | 1350        | 1150        | 60         | 1100       | 1060                   | 1.2       | 80        |
| 42 | MD7 | 1350        | 1150        | 60         | 1100       | 1060                   | 1.2       | 80        |
| 43 | MD7 | <u>1280</u> | 1110        | 30         | 1080       | 1050                   | 1         | 80        |
| 44 | MD7 | <u>1500</u> |             |            |            | HOT ROLLING IMPOSSIBLE |           |           |
| 45 | MD7 | 1350        | <u>1220</u> | 80         | 1100       | 1050                   | 1         | 80        |
| 46 | MD7 | 1350        | 1150        | <u>320</u> | 1100       | 1050                   | 1         | 80        |
| 47 | MD7 | 1350        | 1150        | 110        | <u>980</u> | 1000                   | 1         | 80        |
| 48 | MD7 | 1350        | 1150        | 60         | 1100       | <u>930</u>             | 1         | 60        |
| 49 | MD7 | 1350        | 1150        | 10         | 1130       | <u>1120</u>            | 1         | 90        |
| 50 | MD7 | 1350        | 1150        | 60         | 1100       | 1060                   | <u>12</u> | 80        |
| 51 | MD7 | 1350        | 1150        | 60         | 1100       | 1060                   | 1.2       | <u>45</u> |
| 52 | MD7 | 1350        | 1150        | 60         | 1100       | 1060                   | 1.2       | 80        |
| 53 | MD8 | 1350        | 1150        | 60         | 1100       | 1060                   | 1.2       | 80        |
| 54 | MD8 | 1350        | 1150        | 60         | 1100       | 1060                   | 1.2       | 80        |
| 55 | MD8 | 1350        | 1150        | 60         | 1100       | 1060                   | 1.2       | 80        |
| 56 | MD8 | <u>1280</u> | 1110        | 30         | 1080       | 1050                   | 1         | 80        |
| 57 | MD8 | <u>1500</u> |             |            |            | HOT ROLLING IMPOSSIBLE |           |           |
| 58 | MD8 | 1350        | <u>1220</u> | 80         | 1100       | 1050                   | 1         | 80        |
| 59 | MD8 | 1350        | 1150        | <u>320</u> | 1100       | 1050                   | 1         | 80        |
| 60 | MD8 | 1350        | 1150        | 110        | <u>980</u> | 990                    | 1         | 80        |

| SAMPLE<br>No. | COILING<br>TEMPERATURE<br>(° C.) | PICKLING<br>BATH<br>TYPE     | DECARBURIZED |            |                                          |                                          | GRAIN-ORIENTED ELECTRICAL<br>STEEL SHEET          |                                             |
|---------------|----------------------------------|------------------------------|--------------|------------|------------------------------------------|------------------------------------------|---------------------------------------------------|---------------------------------------------|
|               |                                  |                              | STEEL SHEET  |            | LIGHT-<br>EMITTING<br>INTENSITY<br>RATIO | LIGHT-<br>EMITTING<br>INTENSITY<br>RATIO | MAGNETIC<br>FLUX<br>DENSITY B <sub>8</sub><br>(T) | COATING<br>FILM<br>RESIDUAL<br>RATIO<br>(%) |
|               |                                  |                              | MEASUREMENT  | IMPOSSIBLE |                                          |                                          |                                                   |                                             |
| 31            |                                  | HOT ROLLING B2<br>IMPOSSIBLE |              |            |                                          |                                          |                                                   |                                             |
| 32            | 550                              | B2                           |              |            | 0.40                                     | <u>0.35</u>                              | 1.94                                              | 95                                          |
| 33            | 550                              | B2                           |              |            | 0.40                                     | <u>0.35</u>                              | 1.94                                              | 95                                          |
| 34            | 550                              | B2                           |              |            | 0.40                                     | <u>0.35</u>                              | 1.94                                              | 95                                          |
| 35            | 550                              | B2                           |              |            | 0.40                                     | <u>0.35</u>                              | 1.94                                              | 95                                          |
| 36            | 550                              | B2                           |              |            | 0.40                                     | <u>0.35</u>                              | 1.94                                              | 95                                          |
| 37            | 550                              | B2                           |              |            | 0.40                                     | <u>0.35</u>                              | 1.94                                              | 95                                          |
| 38            | 550                              | B2                           |              |            | 0.40                                     | <u>0.35</u>                              | 1.94                                              | 95                                          |
| 39            | <u>620</u>                       | B2                           |              |            | 0.40                                     | <u>0.35</u>                              | 1.94                                              | 95                                          |
| 40            | 550                              | B1                           |              |            | 0.40                                     | 0.30                                     | 1.95                                              | 90                                          |
| 41            | 550                              | B2                           |              |            | 0.35                                     | 0.20                                     | 1.95                                              | 100                                         |
| 42            | 550                              | <u>B3</u>                    |              |            | <u>0.70</u>                              | <u>0.40</u>                              | 1.94                                              | 60                                          |
| 43            | 550                              | B2                           |              |            | 0.45                                     | 0.23                                     | 1.86                                              | 100                                         |
| 44            | HOT ROLLING B2<br>IMPOSSIBLE     |                              |              |            |                                          |                                          | MEASUREMENT IMPOSSIBLE                            |                                             |
| 45            | 550                              | B2                           |              |            | 0.48                                     | 0.22                                     | 1.92                                              | 100                                         |
| 46            | 550                              | B2                           |              |            | 0.42                                     | 0.20                                     | 1.90                                              | 100                                         |
| 47            | 550                              | B2                           |              |            | 0.45                                     | 0.20                                     | 1.91                                              | 100                                         |
| 48            | 550                              | B2                           |              |            | 0.45                                     | 0.20                                     | 1.88                                              | 100                                         |
| 49            | 550                              | B2                           |              |            | 0.45                                     | 0.20                                     | 1.91                                              | 100                                         |
| 50            | 550                              | B2                           |              |            | 0.45                                     | 0.20                                     | 1.92                                              | 100                                         |
| 51            | 550                              | B2                           |              |            | 0.45                                     | 0.20                                     | 1.92                                              | 100                                         |
| 52            | <u>620</u>                       | B2                           |              |            | 0.45                                     | 0.20                                     | 1.90                                              | 100                                         |
| 53            | 550                              | B1                           |              |            | 0.30                                     | 0.25                                     | 1.94                                              | 95                                          |
| 54            | 550                              | B2                           |              |            | 0.25                                     | 0.15                                     | 1.94                                              | 100                                         |
| 55            | 550                              | <u>B3</u>                    |              |            | <u>0.70</u>                              | <u>0.32</u>                              | 1.93                                              | 50                                          |
| 56            | 550                              | B2                           |              |            | 0.30                                     | 0.20                                     | 1.82                                              | 100                                         |
| 57            | HOT ROLLING B2<br>IMPOSSIBLE     |                              |              |            |                                          |                                          | MEASUREMENT IMPOSSIBLE                            |                                             |
| 58            | 550                              | B2                           |              |            | 0.30                                     | 0.20                                     | 1.82                                              | 100                                         |
| 59            | 550                              | B2                           |              |            | 0.30                                     | 0.20                                     | 1.88                                              | 100                                         |
| 60            | 550                              | B2                           |              |            | 0.30                                     | 0.20                                     | 1.87                                              | 100                                         |

TABLE 5

| SAMPLE<br>No.                         | STEEL<br>TYPE | HOT ROLLING                           |                                    |                             |                                                         |                                          |                                                   |                                             |  |
|---------------------------------------|---------------|---------------------------------------|------------------------------------|-----------------------------|---------------------------------------------------------|------------------------------------------|---------------------------------------------------|---------------------------------------------|--|
|                                       |               | SLAB HEATING<br>TEMPERATURE<br>(° C.) | FINISHING<br>TEMPERATURE<br>(° C.) | STANDBY<br>TIME<br>(SECOND) | ROUGH<br>ROLLING                                        | FINISH<br>ROLLING                        | FINISH<br>ROLLING                                 | COOLING                                     |  |
|                                       |               |                                       |                                    |                             | START<br>TEMPERATURE<br>(° C.)                          | FINISHING<br>TEMPERATURE<br>(° C.)       | STANDBY<br>TIME<br>(SECOND)                       | COOLING<br>RATE<br>(° C./SECOND)            |  |
| 61                                    | MD8           | 1350                                  | 1150                               | 60                          | 1100                                                    | 930                                      | 1                                                 | 60                                          |  |
| 62                                    | MD8           | 1350                                  | 1150                               | 10                          | 1130                                                    | 1120                                     | 1                                                 | 90                                          |  |
| 63                                    | MD8           | 1350                                  | 1150                               | 60                          | 1100                                                    | 1060                                     | 12                                                | 80                                          |  |
| 64                                    | MD8           | 1350                                  | 1150                               | 60                          | 1100                                                    | 1060                                     | 1.2                                               | 45                                          |  |
| 65                                    | MD8           | 1350                                  | 1150                               | 60                          | 1100                                                    | 1060                                     | 1.2                                               | 80                                          |  |
| 66                                    | MD9           | 1350                                  | 1150                               | 60                          | 1100                                                    | 1060                                     | 1.2                                               | 80                                          |  |
| 67                                    | MD9           | 1350                                  | 1150                               | 60                          | 1100                                                    | 1060                                     | 1.2                                               | 80                                          |  |
| 68                                    | MD9           | 1350                                  | 1150                               | 60                          | 1100                                                    | 1060                                     | 1.2                                               | 80                                          |  |
| 69                                    | MD9           | 1280                                  | 1110                               | 30                          | 1080                                                    | 1050                                     | 1                                                 | 80                                          |  |
| 70                                    | MD9           | 1500                                  |                                    |                             | HOT ROLLING IMPOSSIBLE                                  |                                          |                                                   |                                             |  |
| 71                                    | MD9           | 1350                                  | 1220                               | 80                          | 1100                                                    | 1050                                     | 1                                                 | 80                                          |  |
| 72                                    | MD9           | 1350                                  | 1150                               | 320                         | 1100                                                    | 1050                                     | 1                                                 | 80                                          |  |
| 73                                    | MD9           | 1350                                  | 1150                               | 110                         | 980                                                     | 990                                      | 1                                                 | 80                                          |  |
| 74                                    | MD9           | 1350                                  | 1150                               | 60                          | 1100                                                    | 930                                      | 1                                                 | 60                                          |  |
| 75                                    | MD9           | 1350                                  | 1150                               | 10                          | 1130                                                    | 1120                                     | 1                                                 | 90                                          |  |
| 76                                    | MD9           | 1350                                  | 1150                               | 60                          | 1100                                                    | 1060                                     | 12                                                | 80                                          |  |
| 77                                    | MD9           | 1350                                  | 1150                               | 60                          | 1100                                                    | 1060                                     | 1.2                                               | 45                                          |  |
| 78                                    | MD9           | 1350                                  | 1150                               | 60                          | 1100                                                    | 1060                                     | 1.2                                               | 80                                          |  |
| 79                                    | MD10          | 1350                                  | 1150                               | 60                          | 1100                                                    | 1060                                     | 1.2                                               | 80                                          |  |
| 80                                    | MD10          | 1350                                  | 1150                               | 60                          | 1100                                                    | 1060                                     | 1.2                                               | 80                                          |  |
| 81                                    | MD10          | 1350                                  | 1150                               | 60                          | 1100                                                    | 1060                                     | 1.2                                               | 80                                          |  |
| 82                                    | MD10          | 1280                                  | 1110                               | 30                          | 1080                                                    | 1050                                     | 1                                                 | 80                                          |  |
| 83                                    | MD10          | 1500                                  |                                    |                             | HOT ROLLING IMPOSSIBLE                                  |                                          |                                                   |                                             |  |
| 84                                    | MD10          | 1350                                  | 1220                               | 80                          | 1100                                                    | 1050                                     | 1                                                 | 80                                          |  |
| 85                                    | MD10          | 1350                                  | 1150                               | 320                         | 1100                                                    | 1050                                     | 1                                                 | 80                                          |  |
| 86                                    | MD10          | 1350                                  | 1150                               | 110                         | 980                                                     | 990                                      | 1                                                 | 80                                          |  |
| 87                                    | MD10          | 1350                                  | 1150                               | 60                          | 1100                                                    | 930                                      | 1                                                 | 60                                          |  |
| 88                                    | MD10          | 1350                                  | 1150                               | 10                          | 1130                                                    | 1120                                     | 1                                                 | 90                                          |  |
| 89                                    | MD10          | 1350                                  | 1150                               | 60                          | 1100                                                    | 1060                                     | 12                                                | 80                                          |  |
| 90                                    | MD10          | 1350                                  | 1150                               | 60                          | 1100                                                    | 1060                                     | 1.2                                               | 45                                          |  |
| 91                                    | MD10          | 1350                                  | 1150                               | 60                          | 1100                                                    | 1060                                     | 1.2                                               | 80                                          |  |
| GRAIN-ORIENTED ELECTRICAL STEEL SHEET |               |                                       |                                    |                             |                                                         |                                          |                                                   |                                             |  |
| SAMPLE<br>No.                         | STEEL<br>TYPE | DECARBURIZED                          |                                    |                             |                                                         |                                          |                                                   |                                             |  |
|                                       |               | COILING<br>TEMPERATURE<br>(° C.)      | PICKLING<br>BATH<br>TYPE           |                             | STEEL SHEET<br>LIGHT-<br>EMITTING<br>INTENSITY<br>RATIO | LIGHT-<br>EMITTING<br>INTENSITY<br>RATIO | MAGNETIC<br>FLUX<br>DENSITY B <sub>8</sub><br>(T) | COATING<br>FILM<br>RESIDUAL<br>RATIO<br>(%) |  |
|                                       |               | 61                                    | 550                                | B2                          | 0.30                                                    | 0.20                                     | 1.91                                              | 100                                         |  |
| 62                                    |               | 550                                   | B2                                 |                             | 0.30                                                    | 0.20                                     | 1.85                                              | 100                                         |  |
| 63                                    |               | 550                                   | B2                                 |                             | 0.30                                                    | 0.20                                     | 1.91                                              | 100                                         |  |
| 64                                    |               | 550                                   | B2                                 |                             | 0.30                                                    | 0.20                                     | 1.92                                              | 100                                         |  |
| 65                                    |               | 620                                   | B2                                 |                             | 0.30                                                    | 0.20                                     | 1.90                                              | 100                                         |  |
| 66                                    |               | 550                                   | B1                                 |                             | 0.30                                                    | 0.25                                     | 1.95                                              | 100                                         |  |
| 67                                    |               | 550                                   | B2                                 |                             | 0.25                                                    | 0.10                                     | 1.95                                              | 100                                         |  |
| 68                                    |               | 550                                   | B3                                 |                             | 0.65                                                    | 0.35                                     | 1.95                                              | 60                                          |  |
| 69                                    |               | 550                                   | B2                                 |                             | 0.45                                                    | 0.35                                     | 1.79                                              | 100                                         |  |
| 70                                    |               | HOT ROLLING<br>IMPOSSIBLE             |                                    | B2                          | MEASUREMENT IMPOSSIBLE                                  |                                          |                                                   |                                             |  |
| 71                                    |               | 550                                   | B2                                 |                             | 0.25                                                    | 0.10                                     | 1.91                                              | 100                                         |  |
| 72                                    |               | 550                                   | B2                                 |                             | 0.30                                                    | 0.15                                     | 1.89                                              | 95                                          |  |
| 73                                    |               | 550                                   | B2                                 |                             | 0.30                                                    | 0.15                                     | 1.92                                              | 95                                          |  |
| 74                                    |               | 550                                   | B2                                 |                             | 0.25                                                    | 0.10                                     | 1.83                                              | 100                                         |  |
| 75                                    |               | 550                                   | B2                                 |                             | 0.30                                                    | 0.15                                     | 1.85                                              | 100                                         |  |
| 76                                    |               | 550                                   | B2                                 |                             | 0.30                                                    | 0.15                                     | 1.88                                              | 100                                         |  |
| 77                                    |               | 550                                   | B2                                 |                             | 0.30                                                    | 0.15                                     | 1.88                                              | 100                                         |  |
| 78                                    |               | 620                                   | B2                                 |                             | 0.30                                                    | 0.15                                     | 1.89                                              | 100                                         |  |
| 79                                    |               | 550                                   | B1                                 |                             | 0.40                                                    | 0.25                                     | 1.94                                              | 95                                          |  |
| 80                                    |               | 550                                   | B2                                 |                             | 0.35                                                    | 0.20                                     | 1.94                                              | 100                                         |  |
| 81                                    |               | 550                                   | B3                                 |                             | 0.70                                                    | 0.35                                     | 1.94                                              | 65                                          |  |
| 82                                    |               | 550                                   | B2                                 |                             | 0.50                                                    | 0.35                                     | 1.82                                              | 100                                         |  |
| 83                                    |               | HOT ROLLING<br>IMPOSSIBLE             |                                    | B2                          | MEASUREMENT IMPOSSIBLE                                  |                                          |                                                   |                                             |  |
| 84                                    |               | 550                                   | B2                                 |                             | 0.35                                                    | 0.10                                     | 1.89                                              | 100                                         |  |
| 85                                    |               | 550                                   | B2                                 |                             | 0.40                                                    | 0.15                                     | 1.86                                              | 95                                          |  |
| 86                                    |               | 550                                   | B2                                 |                             | 0.35                                                    | 0.15                                     | 1.91                                              | 95                                          |  |
| 87                                    |               | 550                                   | B2                                 |                             | 0.35                                                    | 0.10                                     | 1.84                                              | 100                                         |  |
| 88                                    |               | 550                                   | B2                                 |                             | 0.35                                                    | 0.15                                     | 1.82                                              | 100                                         |  |

TABLE 5-continued

|    |     |    |      |      |      |     |
|----|-----|----|------|------|------|-----|
| 89 | 550 | B2 | 0.40 | 0.15 | 1.87 | 100 |
| 90 | 550 | B2 | 0.35 | 0.15 | 1.88 | 100 |
| 91 | 620 | B2 | 0.35 | 0.15 | 1.88 | 100 |

TABLE 6

| BATH TYPE | PICKLING CONDITION                                                                             |
|-----------|------------------------------------------------------------------------------------------------|
| B1        | 8.5% HCl + 0.4% HNO <sub>3</sub> + SURFACE ACTIVE AGENT, 85° C., 40-SECOND IMMERSION           |
| B2        | 8.5% HCl + 0.4% HNO <sub>3</sub> + NITRATE + SURFACE ACTIVE AGENT, 85° C., 40-SECOND IMMERSION |
| B3        | 8.5% HCl, 85° C., 40-SECOND IMMERSION                                                          |

As illustrated in Table 3 to Table 5, in Samples No. 1, No. 2, No. 27, No. 28, No. 40, No. 41, No. 53, No. 54, No. 66, No. 67, No. 79, and No. 80, because of the slab heating temperature, the hot rolling condition, the cooling condition, the coiling temperature, the holding temperature of the hot-rolled sheet annealing, and the pickling condition each being within the range of the present invention, good results, which were the Cu/Fe light-emitting intensity ratio in the decarburized steel sheet of 0.60 or less and the Cu/Fe light-emitting intensity ratio in the grain-oriented electrical steel sheet of 0.30 or less, were obtained. Among these samples, in Samples No. 2, No. 28, No. 41, No. 54, No. 67, and No. 80, since the pickling was performed in the pickling bath containing a nitrate, good results, which were the Cu/Fe light-emitting intensity ratio in the decarburized steel sheet of 0.40 or less and the Cu/Fe light-emitting intensity ratio in the grain-oriented electrical steel sheet of 0.40 or less, were obtained.

In Samples No. 14 and No. 15, because of the C content being too large, the Cu/Fe light-emitting intensity ratio was large. In Samples No. 3, No. 16, No. 29, No. 42, No. 55, No. 68, and No. 81, because of the pickling condition being outside the range of the present invention, the Cu/Fe light-emitting intensity ratio was large. In Samples No. 4, No. 17, No. 30, No. 43, No. 56, No. 69, and No. 82, because of the slab heating temperature being too low, a desired grain-oriented electrical steel sheet was not able to be obtained. In Samples No. 5, No. 18, No. 31, No. 44, No. 57, No. 70, and No. 83, because of the slab heating temperature being too high, the subsequent hot rolling was not able to be performed. In Samples No. 6, No. 19, No. 32, No. 45, No. 58, No. 71, and No. 84, because of the finishing temperature of the rough rolling being too high, a desired grain-oriented electrical steel sheet was not able to be obtained. In Samples No. 7, No. 20, No. 33, No. 46, No. 59, No. 72, and No. 85, because of the time period between start of the rough rolling and start of the finish rolling being too long, a desired grain-oriented electrical steel sheet was not able to be obtained. In Samples No. 8, No. 21, No. 34, No. 47, No. 60, No. 73, and No. 86, because of the start temperature of the finish rolling being too low, a desired grain-oriented electrical steel sheet was not able to be obtained. In Samples No. 9, No. 22, No. 35, No. 48, No. 61, No. 74, and No. 87, because of the finishing temperature of the finish rolling being too low, a desired grain-oriented electrical steel sheet was not able to be obtained. In Samples No. 10, No. 23, No. 36, No. 49, No. 62, No. 75, and No. 88, because of the finishing temperature of the finish rolling being too high, a desired grain-oriented electrical steel sheet was not able to be obtained. In Samples No. 11, No. 24, No. 37, No. 50, No. 63, No. 76, and No. 89, because of the time period between

finish of the finish rolling and start of the cooling being too long, a desired grain-oriented electrical steel sheet was not able to be obtained. In Samples No. 12, No. 25, No. 38, No. 51, No. 64, No. 77, and No. 90, because of the cooling rate after the finish rolling being too slow, a desired grain-oriented electrical steel sheet was not able to be obtained. In Samples No. 13, No. 26, No. 39, No. 52, No. 65, No. 78, and No. 91, because of the coiling temperature being too high, a desired grain-oriented electrical steel sheet was not able to be obtained.

The invention claimed is:

1. A grain-oriented electrical steel sheet, comprising: a chemical composition comprising in mass %, Si: 1.8% to 7.0%, Cu: 0.03% to 0.60%, and the balance: Fe and impurities, wherein the impurities comprise C; and a primary coating film containing forsterite on a surface of the steel sheet, wherein a Cu/Fe light-emitting intensity ratio at an interface region between the primary coating film and the surface of the steel sheet is 0.30 or less, wherein the Cu/Fe light-emitting intensity ratio is evaluated by the average of (Cu light-emitting intensities/Fe light-emitting intensities), obtained by glow discharge optical emission spectrometry analysis, at respective measurement points in the interface region.
2. A manufacturing method of a grain-oriented electrical steel sheet, comprising:
  - a step of heating a slab in a temperature zone of 1300° C. to 1490° C.;
  - a step of obtaining a hot-rolled steel sheet by performing hot rolling of the slab;
  - a step of coiling the hot-rolled steel sheet in a temperature zone of 600° C. or less;
  - a step of performing hot-rolled sheet annealing of the hot-rolled steel sheet;
  - after the hot-rolled sheet annealing, a step of performing cold rolling and obtaining a cold-rolled steel sheet;
  - a step of performing decarburization annealing of the cold-rolled steel sheet; and
  - after the decarburization annealing, a step of applying an annealing separating agent containing MgO and performing finish annealing, wherein the step of performing the hot rolling includes a step of performing rough rolling with a finishing temperature set to 1200° C. or less and a step of performing finish rolling with a start temperature set to 1000° C. or more and a finishing temperature set to 950° C. to 1100° C., in the hot rolling, the finish rolling is started within 300 seconds after start of the rough rolling, cooling at a cooling rate of 50° C./second or more is started within 10 seconds after finish of the finish rolling,
  - pickling with a holding temperature set to 50° C. or more and a holding time period set to 30 seconds or more is performed in a pickling bath containing a nitric acid, a pickling inhibitor, and a surface active agent after the hot rolling and before finish of the cold rolling, and

**25**

the slab includes a chemical composition comprising, in mass %,  
 C: 0.03% to 0.15%,  
 Si: 1.8% to 7.0%,  
 Mn: 0.02% to 0.30%,  
 S: 0.005% to 0.040%,  
 acid-soluble Al: 0.010% to 0.065%,  
 N: 0.0030% to 0.0150%,  
 Cu: 0.03% to 0.60%,  
 Sn: 0% to 0.5%,  
 Ge, Se, Sb, Te, Pb, or Bi, or an arbitrary combination of these: 0.0005% to 0.030% in total, and the balance: Fe and impurities.

3. The manufacturing method of the grain-oriented electrical steel sheet according to claim 2, wherein the pickling bath further contains a nitrate.

4. A manufacturing method of a decarburized steel sheet for a grain-oriented electrical steel sheet, comprising:  
 a step of heating a slab in a temperature zone of 1300° C. to 1490° C.;  
 a step of obtaining a hot-rolled steel sheet by performing hot rolling of the slab;  
 a step of coiling the hot-rolled steel sheet in a temperature zone of 600° C. or less;  
 a step of performing hot-rolled sheet annealing of the hot-rolled steel sheet; 25  
 after the hot-rolled sheet annealing, a step of performing cold rolling and obtaining a cold-rolled steel sheet; and a step of performing decarburization annealing of the cold-rolled steel sheet; wherein  
 the step of performing the hot rolling includes a step of performing rough rolling with a finishing temperature

5

10

15

20

25

30

**26**

set to 1200° C. or less and a step of performing finish rolling with a start temperature set to 1000° C. or more and a finishing temperature set to 950° C. to 1100° C., in the hot rolling, the finish rolling is started within 300 seconds after start of the rough rolling,

cooling at a cooling rate of 50° C./second or more is started within 10 seconds after finish of the finish rolling,

pickling with a holding temperature set to 50° C. or more and a holding time period set to 30 seconds or more is performed in a pickling bath containing a nitric acid, a pickling inhibitor, and a surface active agent after the hot rolling and before finish of the cold rolling, and the slab includes a chemical composition comprising, in mass %

C: 0.03% to 0.15%,  
 Si: 1.8% to 7.0%,  
 Mn: 0.02% to 0.30%,  
 S: 0.005% to 0.040%,  
 acid-soluble Al: 0.010% to 0.065%,  
 N: 0.0030% to 0.0150%,  
 Cu: 0.03% to 0.60%,  
 Sn: 0% to 0.5%,  
 Ge, Se, Sb, Te, Pb, or Bi, or an arbitrary combination of these: 0.0005% to 0.030% in total, and the balance: Fe and impurities.

5. The manufacturing method of the decarburized steel sheet for a grain-oriented electrical steel sheet according to claim 4, wherein

the pickling bath further contains a nitrate.

\* \* \* \* \*